

# UNITED STATES PATENT OFFICE.

PETER PETERSON, OF PHILADELPHIA, PENNSYLVANIA.

## WATER-PROOF FABRIC.

SPECIFICATION forming part of Letters Patent No. 227,573, dated May 11, 1880.

Application filed January 21, 1880.

*To all whom it may concern:*

Be it known that I, PETER PETERSON, of the city and county of Philadelphia, in the State of Pennsylvania, have invented certain new and useful Improvements in Waterproofing and Preserving Fabrics, of which improvements the following is a specification.

The object of my invention is to preserve textile fabrics, specially canvas and goods analogous thereto, from the deteriorating effects of water and dampness; and my improvements consist in fabrics treated with certain primary and secondary waterproofing compositions, all as hereinafter more fully set forth.

To carry out my invention the canvas or other fabric which is to be waterproofed is coated first with a primary and afterward with a secondary composition, the ingredients and proportions of which compositions are as follows: Assuming that a sufficient quantity is desired to cover about five hundred square yards of material, the primary composition consists of seventeen pounds scalded rye-flour, one and a half pound burnt alum, and six gallons water, the water being heated to the boiling-point and maintained thereat until the rye-flour and alum are thoroughly mixed and dissolved.

The primary composition is applied to the material to be waterproofed by a brush or other convenient means, and the material is then dried either by natural or artificial heat, as may be found most desirable.

A corresponding quantity of the secondary

composition consists of twenty-four gallons 35 linseed-oil, three pounds litharge, forty-five and a half pounds American ocher, (or an equivalent quantity of other earth paint, such as Spanish brown or Venetian red,) and one and a half pound melted rosin soap, these ingredients being thoroughly mixed and incorporated together.

A coating of the secondary composition is applied, most conveniently by means of a brush, to one or both sides of the fabric which 45 has been treated with the primary composition, and as soon as the same is dry the operation is complete, and the fabric will be found to fully resist the decay or mildew induced by exposure to water or a damp atmosphere, 50 as well as the attacks of moths, without becoming hard or stiff and without developing any tendency in the preservative compositions to be worn or washed out of its texture.

I claim as my invention and desire to secure 55 by Letters Patent—

A new article of manufacture, consisting of canvas or other textile fabric having a primary coating or layer of a sizing composition, consisting of scalded rye-flour and burnt alum 60 dissolved in water, and a secondary coating or layer of linseed-oil, litharge, earth paint, and rosin soap, as described.

PETER PETERSON.

Witnesses:

J. SNOWDEN BELL,  
W. K. SHRYOCK.